

Oct. 8, 1929.

N. H. ADAMS

1,731,218

ELECTRICAL CONDUCTOR

Filed Oct. 5, 1922

Fig. 1.



Fig. 2.



Fig. 3.



Inventor:  
Nathan H. Adams,

by *Alexander Lutz*  
His Attorney

## UNITED STATES PATENT OFFICE

NATHAN H. ADAMS, OF SCHENECTADY, NEW YORK, ASSIGNOR TO GENERAL ELECTRIC COMPANY, A CORPORATION OF NEW YORK

## ELECTRICAL CONDUCTOR

Application filed October 5, 1922. Serial No. 592,597.

The present invention comprises an improved terminal for flexible conductors which consist of strands of fine wires. It is the object of my invention to provide a strong, 5 rugged terminal to which a good electrical connection may be made without locally overheating, or otherwise injuring the individual wires of the flexible strands.

Heretofore, difficulties have been encountered by the weakening and embrittling of stranded or braided conductors by the use of fluxes when welding, soldering or brazing terminals to conductors. When such operations are carried out in the open air copper 10 wires become oxidized and in the presence of reducing gas, copper becomes brittle. As stranded conductors are particularly intended to be used in apparatus such as circuit breakers in which conductors frequently are 15 subjected to motion, brittleness may soon lead to a break which may cause an expensive shutdown of large apparatus.

In accordance with my invention, I have provided a terminal conductor by causing the 20 wires constituting a stranded conductor to be compacted or welded together by pressure to form a solid bar or plate with the aid of a small quantity of easily fusible metal having preferably a moderate alloying affinity for 25 said wires. For example, in order to bind together under pressure fine copper wires to form a dense, solid metal, I employ a small quantity of lead-tin alloy in which lead preponderates and the tin is in amount sufficient 30 only to cause the alloy to adhere to the surface of the copper.

The accompanying drawing illustrates, in 35 Figs. 1 and 2, a stranded conductor assembled in a press with sheets of binder metal, and Fig. 3 shows in perspective the finished article.

The stranded ribbon-shaped conductors 40 of Fig. 1 consist of fine copper wires which, for example, may be about 10 mils in diameter. Between the strands are placed wafers 45 of an easily fusible metal having a moderate alloying affinity for copper. For example, I have used with success an alloy of nine parts lead and one part tin, although those proportions may be varied considerably. This al-

loy has a melting point of about 290° C. The wafers 5 may be about two mils in thickness. An alloy of this constitution is not suitable for ordinary soldering but the high pressure and high temperature conditions of the present process renders the alloy capable of causing the copper wires to be consolidated into a compact mass. The parts when assembled are placed between the members 6, 7 of a mold heated under a pressure sufficiently high to 55 melt the wafers 5 and to soften the copper. I may use for this purpose a press adapted to convey a heating current through the mass. In the drawing, I have indicated diagrammatically electric terminals 8, 9 by which 60 pressure may be applied. These terminals are connected to conductors 10, 11 preferably including between one of the mold members and the adjoining terminal a strip of material of relatively high resistance, for example 65 a layer 12 consisting of graphite or carbon. A pressure of about two thousand pounds to the square inch ordinarily is satisfactory for 70 the welding operation.

The temperature suitable for this compression and welding step ordinarily will lie within the limits of about 750 to 950° C., depending on the density desired in the terminal. Most commonly I use a temperature of about 75 850° C. At this temperature which approaches the softening temperature of copper, the alloy 5 is highly fluid, so that to a large degree it escapes from the mass and is vaporized. Apparently the alloy acts as a 80 flux to put the metal surfaces into proper condition for welding. Oxide on the surface of the copper wires is removed by the melted flux metal. Oxidized copper may be welded as readily as clean, unoxidized copper.

The welded portion 13 of the conductor 85 may be machined as shown in Fig. 3 to remove surface inequalities. The portion 13 presents to the unaided eye the appearance of a sound homogeneous metal and indeed, has substantially the properties of homogeneous 90 copper. Under the microscope it can be observed to consist of a densely compacted mass in which the original wires or other components are still detectable, in most cases surrounded by a film of alloy.

The compressed mass becomes more dense and homogeneous as the pressure and temperature of the operation are raised.

What I claim as new and desire to secure  
5 by Letters Patent of the United States, is:—

1. An article of manufacture comprising a plurality of members of metal united into a compact, unitary mass and a film of binder metal located in interstices between said members, said binder metal having insufficient alloying affinity for said members to materially attack the surface thereof but being capable of promoting welding of said members under pressure at a temperature approximating the  
10 melting point of said members.
2. An electrical conductor comprising in part a multiplicity of flexible wires and in part a solid bar or plate, said plate comprising a continuation of said wires welded together and containing dispersed between said wires a film of alloy melting at about one-third the softening temperature of the wires.  
20
3. An article of manufacture comprising in part a plurality of filamentary copper wires and in part a substantially solid mass of metal constituted by said wires joined to each other by a film of alloy of lead and tin in which the tin is in amount sufficient to cause the alloy to adhere to the surface of  
25 the copper wires to promote a welding operation.
4. An article of manufacture comprising a plurality of copper filaments and a solid, machinable bar continuous therewith and  
30 having substantially the mechanical properties of a bar of copper of equal size, said bar comprising said filaments joined to each other by an intervening film of binder metal consisting largely of lead and in part of a metal  
35 alloyable with copper.
5. An article of manufacture comprising a bundle of filamentary wires consisting of copper compacted to form a solid mass, said wires being in part welded to each other and  
40 in part joined to each other by a film of alloy which melts at a much lower temperature than the wires and which is present in such small proportion that said mass has substantially the properties of homogeneous copper.
6. An article of manufacture comprising a multiplicity of separate members associated in a densely compacted state, said members being joined to one another by welding and  
45 by a film of alloy having a slight alloying affinity for said members into a mass having the appearance to the unaided eye of sound, homogeneous metal and which when magnified can be seen to comprise distinct component members.  
50
- 60 In witness whereof, I have hereunto set my hand this 4th day of October, 1922.

NATHAN H. ADAMS.